

# UNITED STATES PATENT OFFICE.

CHARLES E. SWETT, OF BROOKLINE, MASSACHUSETTS, ASSIGNOR TO ARTHUR D. LITTLE, INCORPORATED, OF CAMBRIDGE, MASSACHUSETTS, A CORPORATION OF MASSACHUSETTS.

## STENCIL-BLANK.

1,316,067.

Specification of Letters Patent. Patented Sept. 16, 1919.

No Drawing.

Application filed March 15, 1919. Serial No. 282,840.

*To all whom it may concern:*

Be it known that I, CHARLES E. SWETT, a citizen of the United States, residing at Brookline, in the county of Norfolk and 5 State of Massachusetts, have invented certain new and useful Improvements in Stencil-Blanks, of which the following is a specification.

The present invention relates primarily 10 to the manufacture of stencil blanks. For many years stencil blanks have been made from thin, long fibered tissue paper impregnated with an ink-resisting material. When a stencil is made from a blank so 15 prepared, a blow by the type of a stencil cutting machine, for example a typewriting machine, ruptures the film of impregnating ink-resisting material while leaving the fibers mostly unruptured to serve as bridges 20 to support parts of letters like the center of the letter O or the inclosed parts of letters, for example, the capital letter B.

One of the earlier stencil blanks employed a filling material of wax, usually in practice 25 what is known in commerce as paraffin wax. This is capable of making a useful stencil, but because of the brittleness of wax at relatively low temperatures accidental rupture, due to careless handling, may take place 30 and such rupture permit the ink to penetrate, which is of course undesirable. Another objection to the wax impregnated stencil blank is that its life when made in a stencil permits a relatively smaller number 35 of copies to be secured than when other impregnating material is used.

Other matter than wax is employed as 40 film material in the art; some form of protein, as for example gelatin or casein, is applied mixed with glycerin or other hygroscopic material, to prevent the warping of the stencil when dried. The protein is usually rendered insoluble after application 45 by the use of soluble chromium compounds or by alum or preferably by formaldehyde.

To apply a water solution to tissue paper is not easy mechanically. The paper when wet with water will not support its own weight except in small pieces. If larger 50 pieces of paper are used, they must have some kind of mechanical support when wet.

When it is desired to make a stencil from a blank prepared from coagulated protein, it must be dampened with water before the 55 operation of cutting. If much time is oc-

cupied in cutting or in very dry weather, the uncut part of the sheet may have to be taken from the machine for the purpose of again dampening the uncut portion. The subsequent realinement in the machine is 60 inherently troublesome.

It is the main object of the present invention to produce a stencil blank which, having a continuous and homogeneous film, will stand considerable wear without liability 65 to crack or receive other injury at all ordinary temperatures, which is not liable to deterioration from age and need not be dampened before the operation of cutting the stencil. 70

I have discovered that an improved stencil blank may be made from thin, long fibered tissue paper if instead of impregnating with wax on the one hand or with protein and hygroscopic material on the other, I employ 75 a composition for filling, which is either wholly or in large part composed of aluminum soap of fatty acids. The aluminum soaps of some fatty acids (for instance oleic and palmitic acid) are insoluble in water 80 and possess a rubber like quality. They will dissolve in mineral oil and their likeness to unvulcanized rubber is still more marked in such solution.

In practice I preferably use higher fatty 85 acids than oleic, for instance palmitic acid. I have made good stencil blanks by dissolving the aluminum soap made from palm oil in gasoline, impregnating the paper with the solution and then permitting the gasoline 90 to evaporate. The quality of the blanks may be improved by adding to the gasoline solution of the aluminum soap, some mineral oil nonvolatile at ordinary temperatures. While there is of course some latitude in the selection of the proportions of the aluminum soap and the heavy mineral oil, I have found that the mixture of five parts of the aluminum soap and about one part of the heavy mineral oil gives excellent 95 results. Gasoline is used only as a solvent. When it evaporates from the solution after application, the aluminum soap and mineral oil are in solid solution and the compound makes an excellent continuous 100 and homogeneous ink-proof film, cuts in distinct lines and the stencil cut is non-healing. 105

By applying solutions containing no water, many of the usual manufacturing diffi- 110

culties are avoided. The aluminum soap film material is water-proof and the stencil blank does not require moistening before cutting.

5 I suggest the following steps for making the solution:

First, I make a neutral water-soluble soap from the desired fatty materials. This is precipitated from a water solution of an 10 aluminum salt, conveniently aluminum sulfate.

Second. The aluminum soap is washed and dried, preferably in the dark and at a 15 temperature insufficient to melt the aluminum soap.

Third. The dry aluminum soap (approximately dry) is covered with gasoline and allowed to swell. It is then warmed and 20 stirred. At this stage, or at any previous one, the mineral oil may be added.

It is understood that this is not the only way of making the compound or solution, but for practical purposes it is probably the best.

25 I claim:

1. A stencil blank made from long fibered tissue paper impregnated with an aluminum

soap of fatty acids comprising the greater part of the filling material.

2. A stencil blank made from long fibered 30 tissue paper impregnated with a compound containing aluminum soap of fatty acids and a fluid hydrocarbon of the paraffin series, the former comprising the greater part of the filling material. 35

3. A stencil blank made from long fibered tissue paper impregnated with an aluminum soap of fatty acids derived principally from palmitic acid, said soap comprising the greater part of the filling material. 40

4. A stencil blank made from long fibered tissue paper impregnated with a compound containing aluminum soap of fatty acids and a fluid hydrocarbon of the paraffin series, the former being derived principally 45 from palmitic acid and comprising the greater part of the filling material.

5. A stencil blank made from long fibered tissue paper impregnated with a compound containing the aluminum soap of palmitic acid and mineral oil, the former comprising 50 over one half the mixture.

In testimony whereof, I affix my signature.  
CHARLES E. SWETT.